

Nov. 27, 1973

F. C. MCCOY ET AL

3,775,324

LUBRICATING OIL COMPOSITION

Filed June 16, 1971

FOAM HEIGHT DURING T-12 LOW ENERGY CYCLING TEST



# United States Patent Office

3,775,324

Patented Nov. 27, 1973

1

Patent No. 3,775,324

## LUBRICATING OIL COMPOSITION

Frederic C. McCoy, Beacon, Arthur W. Godfrey, Fishkill, and Robert E. Reid, Glenham, N.Y., assignors to Texaco Inc., New York, N.Y.

Filed June 16, 1971, Ser. No. 153,534

Int. Cl. C10m 1/28

U.S. Cl. 252—54.6

8 Claims

### ABSTRACT OF THE DISCLOSURE

Lubricant composition having improved anti-foaming properties comprising a mineral lubricating oil and containing an anti-foam amount of perfluoroalkylpolyether.

### BACKGROUND OF THE INVENTION

In many applications, mineral lubricating oil compositions are employed as functional fluids or power transmitting fluids. Examples of this are automatic transmission units, pumps and hydraulic equipment. In such uses, the fluids are pumped or circulated at high speeds which causes the entrainment of air in the fluid with the resultant production of considerable amounts of foam.

Foam in a functional fluid is highly detrimental to the operation of an automatic transmission or a hydraulic device. The foaming characteristics of oil compositions is recognized as a serious problem and industry-adopted specifications have been set on this lubricating oil property. Functional fluids must pass the foam test standards before they will be qualified for hydraulic or transmission service.

The foaming tendency of a lubricating oil composition is intensified by the presence of many additives conventionally employed in lubricating oils. The problem is generally further aggravated by the joint use of a number of additives in the same lubricant composition and by increasing concentrations of the additives.

The foaming tendency of many commercial functional fluids is controlled by the use of alkyl silicone fluids which are effective anti-foam additives in many applications. The silicone anti-foam additives, however, are not effective in some applications for functional fluids.

### SUMMARY OF THE INVENTION

The lubricating oil composition comprises a mixture of hydrocarbons of lubricating viscosity containing a minor, foam-inhibiting amount of perfluoroalkylpolyether. More specifically, the lubricating oil composition will comprise a hydrocarbon base oil having an SUS viscosity at 100° F. from 50 to 2,000 containing from about 1 to 500 parts per million by weight of a perfluoroalkylpolyether corresponding to the formula:



in which  $n$  has a value providing an average molecular weight for the perfluoroalkylpolyether ranging from about 2,000 to 7,000.

FIG. 1 is an illustration of foam heights produced during an automatic transmission test using different anti-foam additives.

The mineral oil base for the lubricating oil composition of the invention can be a paraffinic base, naphthenic base or a mixed paraffinic-naphthenic base distillate or residual oil. Paraffinic base distillate lubricating oil fractions are preferred for the formulation of higher quality lubricating oils. Such a lubricating oil base will usually have been subjected to solvent refining to improve its oxidation stability and viscosity temperature properties as well as solvent dewaxing to remove wax components and thus reduce the pour point of the oil. Generally, mineral lubricating oils fractions of interest for this in-

2

vention have an SUS viscosity at 100° F. between 50 and 2,000 with the preferred mineral lubricating base oils having an SUS viscosity at 100° F. ranging from about 70 to 300.

5 The perfluoroalkylpolyethers of the invention correspond to the formula:



in which  $n$  has a value providing an average molecular weight for the perfluoroalkylpolyether ranging from about 2,000 to 7,000. This molecular weight range will correspond to values for  $n$  of about 10 to 41. The preferred perfluoroalkylpolyethers are those in which the average molecular weight ranges from about 3,000 to about 5,500 which molecular weights correspond to values for  $n$  of about 17 to 32, respectively. Specific examples of effective perfluoroalkylpolyethers are described below.

### EXAMPLE I

20 A perfluoroalkylpolyether having the formula:



and having an average molecular weight of 4,500 corresponding to a value for  $n$  of about 26. This perfluoroalkylpolyether has a viscosity in centistokes at 100° F. of 85 and at 0° F. of 6,900, and an approximate boiling range at 0.8 mm. Hg of 440–485° F.

### EXAMPLE II

25 A perfluoroalkylpolyether having the formula:



and having an average molecular weight of approximately 2,000 corresponding to a value for  $n$  of about 11. This perfluoroalkylpolyether has a viscosity in centistokes at 100° F. of 18 and at 0° F. of 550 and an approximate boiling range at 0.8 mm. Hg of 290–365° F.

### EXAMPLE III

30 A perfluoroalkylpolyether having the formula:



and having an average molecular weight of about 7,000 corresponding to a value for  $n$  of about 41. This perfluoroalkylpolyether has a viscosity in centistokes at 100° F. of 495 and at 210° F. of 43, and a vapor pressure at 700° F. of about 80 mm. of Hg.

35 Functional fluids or lubricating oil compositions of the invention will generally contain a variety of known lubricating oil additives. The perfluoroalkylpolyether additive of the invention is outstanding for providing antifoam properties in functional fluids containing a variety of lubricating oil additives in substantial concentrations.

40 Additives which can be employed in the lubricating oil composition of the invention include but are not limited to the alkylated diarylamines, as illustrated by U.S. Pat. 3,414,618, the zinc dithiophosphates as illustrated by U.S. Pats. 2,344,395 and 3,293,181, the mono-hydroxyalkyl hydrocarbyl thiophosphonates as illustrated by U.S. Pats. 3,135,729 and 3,272,744, the alkali metal sulfonates as illustrated by U.S. Pat. 3,537,996, the alkenyl succinic acid or anhydride polyalkylene polyamine reaction products as illustrated by U.S. Re. 26,433 and U.S. Pat. 3,131,150 and the polymethacrylate polymers as illustrated by U.S. Pats. 2,737,496 and 2,471,959. The disclosures in these 45 references are incorporated in the present invention.

45 A very small concentration of the perfluoroalkylpolyether is effective to produce an anti-foam or foam-resistant lubricating oil composition. Generally, the concentration of the perfluoroalkylpolyether will range from about 1 to 500 parts per million. The preferred concentration of the perfluoroalkylpolyether is from about 5 to 100 parts per million.

The anti-foam properties of a series of lubricating oil composition was determined in the ASTM Foam Test, D-892. According to this test the foam volume is determined at the end of five (5) minutes blowing with air and again after standing for an additional ten (10) minutes in each of the three test steps or sequences, namely sequence I run at 75° F., sequence II run at 200° F. and sequence III rerun of the same sample used in sequence II and run at 75° F. The results of these tests are set out in Table I below.

TABLE I.—FOAM INHIBITING PROPERTIES OF PERFLUOROALKYL POLYETHER

|                                                                | RUN |     |      |      |     |    |      |      |
|----------------------------------------------------------------|-----|-----|------|------|-----|----|------|------|
|                                                                | 1   | 2   | 3    | 4    | 5   | 6  | 7    | 8    |
| <b>Composition (wt. percent):</b>                              |     |     |      |      |     |    |      |      |
| Paraffinic mineral oil SUS visc. at 100° F. of 335             | 100 | 100 | 98.3 | 98.3 | 50  | 50 | 49.0 | 49.0 |
| Paraffinic mineral oil, SUS visc. at 210° F. of 160            |     |     |      |      | 50  | 50 | 49.0 | 49.0 |
| Basic barium alkylphenolate (16.5% barium) (50% conc. in oil)  |     |     | 1.7  | 1.7  |     |    |      |      |
| Overbased calcium sulfonate, 300 TBN (12% Ca)                  |     |     |      |      |     |    | 2.0  | 2.0  |
| Perfluoroalkyl polyether, or Example I, p.p.m.                 | 20  |     | 20   |      | 20  |    |      | 20   |
| <b>ASTM foam test</b>                                          |     |     |      |      |     |    |      |      |
| I II III I II III I II III I II III I II III I II III I II III |     |     |      |      |     |    |      |      |
| Vol. foam after 5 min., blowing, cc.....                       | 530 | 30  | 420  | 0    | 30  | 0  | 660  | 600  |
| Vol. foam after 10 min., standing cc.....                      | 0   | 0   | 0    | 0    | 0   | 0  | 420  | 10   |
|                                                                | 590 | 30  | 20   | 500  | 310 | 60 | 330  | 0    |
|                                                                | 0   | 0   | 350  | 20   | 0   | 10 | 0    | 0    |
|                                                                | 0   | 0   | 0    | 0    | 0   | 0  | 0    | 0    |
|                                                                | 570 | 710 | 490  | 30   | 0   | 0  | 20   | 0    |
|                                                                | 590 | 440 | 440  | 0    | 0   | 0  | 0    | 0    |

The foregoing data illustrates outstanding improvements in the anti-foam property of both simple and additive containing mineral lubricating oil compositions containing the perfluoroalkylpolyethers of the invention.

The anti-foam properties of a variety of mineral lubricating oil compositions containing relatively high concentrations of convention lubricating oil additives was determined in the Detroit Transmission Dynamic Foam Test developed by the Hydra-matic Division of General Motors Corporation. This test simulates the foaming caused in commercial automatic transmissions through the use of a pump, a circulating system, a heater and an agitating device. The test fluid is maintained at temperature of 275° F. The fluids fail this test if the foam height exceeds  $\frac{3}{8}$  (three-eighths) of an inch or if the foam collapse time exceeds (23) twenty-three seconds. The results of this test are set out in Table II below which compares the anti-foam properties of the lubricants of the invention with similar lubricating oil compositions.

Foam production in the fluid without the perfluoroalkylpolyester, measured by height in inches of foam produced, was four to five times as high as that produced by the fluid of Run 15. This test illustrates an unexpected improvement in the antifoam properties realized by the fluid compositions of this invention.

All of the foregoing tests show the outstanding anti-foam property of the functional fluids of the invention. The improvement in this property is essential for functional fluid compositions containing relatively high pro-

portions of additives in order to qualify the fluids for automatic transmission and central hydraulic system service.

We claim:

1. A lubricating oil composition consisting essentially of a major amount of mineral oil in the lubricating oil range having an SUS viscosity at 100° F. between 50 and 2,000 containing from about 1 to 500 parts per million by weight of a perfluoroalkylpolyether having the formula:



in which  $n$  has a value providing an average molecular weight for the perfluoroalkylpolyether ranging from about 2,000 to 7,000.

2. A lubricating oil composition according to claim 1 in which said perfluoroalkylpolyether has an average molecular weight ranging from about 3,000 to 5,500.

3. A lubricating oil composition according to claim 1 in which said perfluoroalkylpolyether has an average molecular weight of about 4,500.

4. A lubricating oil composition according to claim 1

TABLE II

| Composition (wt. percent):                                                                  | Run   |       |       |       |       |       |       |
|---------------------------------------------------------------------------------------------|-------|-------|-------|-------|-------|-------|-------|
|                                                                                             | 9     | 10    | 11    | 12    | 13    | 14    | 15    |
| 1. Solvent refined naphthene base mineral oil having an SUS viscosity at 100° F. of 50..... | 42.00 | 45.00 | 42.00 | 42.00 | 42.00 | 45.00 | 42.00 |
| 2. Paraffinic mineral oil having an SUS viscosity at 100° F. of 100.....                    | 44.74 | 41.00 | 44.74 | 44.74 | 45.44 | 41.00 | 45.44 |
| 3. Polymethacrylate viscosity index improver.....                                           | 8.00  | 8.00  | 8.00  | 8.00  | 8.00  | 8.00  | 8.00  |
| 4. Additive concentrate.....                                                                | 15.26 | 6.00  | 15.26 | 15.26 | 8.56  | 6.00  | 8.56  |
| 5. Silicone solution, p.p.m.....                                                            | 150   | 150   | 150   | 330   | 150   | 150   | 25    |
| 6. Perfluoroalkyl polyether of Example I, <sup>7</sup> p.p.m.....                           |       |       |       |       |       |       | 100   |

<sup>1</sup> Blend of conventional lubricant additives.  
<sup>2</sup> Commercial lubricant additive blend.  
<sup>3</sup> Second blend of conventional lubricant additives.  
<sup>4</sup> 12 wt. percent solution in kerosene of silicone fluid of 100,000 cs. at 77° F.  
<sup>5</sup> 12 wt. percent solution in kerosene of silicone fluid of 60,000 cs. at 77° F.  
<sup>6</sup> 5.6 wt. percent solution in kerosene of silicone fluid of 1,000,000 cs. at 77° F. with dispersant.

The foregoing data illustrates the exceptional improvement realized in the anti-foam property of fully formulated lubricating oil compositions employing the perfluoroalkylpolyether anti-foamant additive of the invention.

The fluid of Run 15 in Table II and a similar fluid without the perfluoroalkylpolyether anti-foamant but containing a conventional 100,000 cs. silicone anti-foamant were run in the T-12 Low Energy Cycling Test and the foam produced was monitored throughout the test. The results of this test are illustrated in the accompanying Figure 1.

in which said perfluoroalkylpolyether has an average molecular weight of about 2,000.

5. A lubricating oil composition according to claim 1 containing in addition from about 0.01 to 20 weight percent of a foam-promoting mineral lubricating oil additive.

6. A lubricating oil composition according to claim 1 containing from about 0.1 to 10 percent of a polymethacrylate viscosity index improver.

7. A lubricating oil composition according to claim 1 containing from about 5 to 100 parts per million of said perfluoroalkylpolyether.

<sup>7</sup> As a solution 10 grams diluted to 100 g. in trifluorotrichloroethane.

D.T.D. FOAM TEST

| 275° F. foam height, in..... | ½  | ⅓  | ⅔  | ⅔  | 0 | 0 | 0 |
|------------------------------|----|----|----|----|---|---|---|
| Collapse time, sec.....      | 37 | 55 | 37 | 30 |   |   |   |

3,775,324

5

8. A lubricating oil composition according to claim 1 in which said mineral oil has an SUS viscosity at 100° F. from 70 to 300.

6

2,515,115 7/1950 Davis et al. ----- 252—54.6  
2,915,471 12/1959 Lorensen ----- 252—54.6 X

PATRICK P. GARVIN, Primary Examiner

References Cited

UNITED STATES PATENTS

5

U.S. Cl. X.R.

3,445,392 5/1969 Gumprecht et al. ----- 252—54  
3,597,359 8/1971 Smith ----- 252—78  
252—54, 33.4, 42.7, 78